

# UNITED STATES PATENT OFFICE.

PAUL W. AVERY AND EUGENE C. KNOWLES, OF DEADWOOD, SOUTH DAKOTA.

## PROCESS OF TREATING PRECIOUS-METAL-BEARING MATERIALS.

963,111.

Specification of Letters Patent.

Patented July 5, 1910.

No Drawing.

Application filed October 19, 1908. Serial No. 458,471.

*To all whom it may concern:*

Be it known that we, PAUL W. AVERY and EUGENE C. KNOWLES, citizens of the United States, residing at Deadwood, in the county 5 of Lawrence and State of South Dakota, have invented certain new and useful Improvements in Processes of Treating Precious-Metal-Bearing Materials, of which the following is a specification.

10 Our invention relates to an improvement in the art of treating precious metal bearing materials, particularly those ores or tailings which contain precious metals incased in sulfids, and it consists in subjecting the 15 above specified precious metal bearing material to the action of the carbonates and hydroxids of the alkali metals, or the alkaline earth metals, or in the presence of atmospheric air, or other oxidizing agent under 20 pressure, for the purpose of liberating the precious metals from the aforesaid sulfids and subsequently bringing a dissolving solution in contact with said material.

In the usual method of treating ore, tailings, or like precious metal bearing materials 25 with alkaline cyanogen solutions there is often present in the material which is being treated complex sulfids which either by reason of their chemical composition exercise 30 a deterrent effect on the dissolution of the precious metals, or by reason of precious metals being incased therein impede the dissolution of the precious metal by the dissolving solution.

35 Now we have discovered that if before treatment with the dissolving solution the said sulfids in the materials treated are decomposed by the elimination of sulfur much more efficient dissolution of the precious 40 metals will result. This is accomplished preferably by treating the particles of the precious metal bearing material in the presence of a suitable oxidizing agent, such as air under pressure, with a basic solution which 45 will decompose the sulfids present in the mass, such as a solution of carbonates, or hydroxids of the alkali metals or alkaline earth metals, or a solution composed of a combination of two or more of the same.

50 The process may be carried out in any form of container in which a contact may be maintained between the basic solution, any desirable oxidizing agent and the particles containing the precious metals, and in practice we employ commercial caustic soda as 55 the most suitable reagent, for the reason that

it is obtainable in sufficient quantities at low cost. Moreover the caustic soda can be regenerated by the addition of the very cheap chemical calcium hydroxid, by agitation 60 with the stock working solution of sodium hydroxid, carbonate, sulfate, etc. After the decomposition has taken place, the solution is then removed from the material in any convenient manner and the latter is subjected 65 to any approved treatment for recovering the precious metals. The effect of this treatment is similar to that resultant from roasting an ore, namely, an oxidized product results, which is chemically and physically 70 different from its original state in the ore.

We claim as our invention:

1. The method of treating precious metal bearing materials containing sulfids, which consists in treating said material in the presence of a suitable oxidizing agent, with a basic solution which will sufficiently decompose the sulfids present therein to enable the precious metals to be readily separated therefrom, then removing the resultant solution and subsequently recovering the precious metals from said material in any convenient manner.

2. The method of treating precious metal bearing materials containing sulfids, which consists in treating said material in the presence of a suitable oxidizing agent, with a solution containing alkali-metal which will sufficiently decompose the sulfids present therein to enable the precious metals to be 80 readily separated therefrom, then removing the resultant solution and subsequently recovering the precious metals from said material in any convenient manner.

3. The method of treating precious metal bearing materials containing sulfids, which consists in treating said material in the presence of a suitable oxidizing agent, with a solution containing a mixture of a carbonate and a hydroxid of an alkali-metal which 90 will sufficiently decompose the sulfids present therein to enable the precious metals to be readily separated therefrom, then removing the resultant solution and subsequently recovering the precious metals from said 95 material in any convenient manner.

4. The method of treating precious metal bearing materials, containing sulfids, which consists in treating said material in the presence of a suitable oxidizing agent with a solution containing a hydroxid of an alkaline earth metal which will sufficiently decom- 110

pose the sulfids present therein, to enable the precious metals to be readily separated therefrom, then removing the resultant solution, and subsequently recovering the 5 precious metals from said material in any convenient manner.

5. The method of treating precious metal bearing materials containing sulfids, which consists in treating said material in the presence 10 of a suitable oxidizing agent, with a solution of caustic soda which will sufficiently decompose the sulfids present therein to enable the precious metals to be readily separated therefrom, then removing the resultant 15 solution and subsequently recovering the precious metals from said material in any convenient manner.

6. The method of treating precious metal bearing materials, containing sulfids, which 20 consists in treating said material in the presence of a suitable oxidizing agent with a solution containing a carbonate of an alkali metal and caustic soda, removing the resultant solution, and subsequently recovering 25 the precious metals from said material in any convenient manner.

7. The method of treating precious metal bearing materials containing sulfids, which consists in agitating said material with a 30 suitable gaseous oxidizing agent under pressure in a basic solution which will sufficiently decompose the sulfids present therein to enable the precious metals to be readily separated therefrom, then removing the resultant 35 solution and subsequently recovering the precious metals from said material in any convenient manner.

8. The method of treating precious metal bearing materials containing sulfids, which 40 consists in agitating said material with a suitable gaseous oxidizing agent, under pressure in a solution containing alkali metal which will sufficiently decompose the sulfids present therein to enable the precious 45 metals to be readily separated therefrom, then removing the resultant solution and subsequently recovering the precious metals from said material in any convenient manner.

50 9. The method of treating precious metal bearing materials containing sulfids, which consists in agitating said material with a suitable gaseous oxidizing agent under pressure in a solution containing a mixture of 55 a carbonate and a hydroxid of an alkali-metal which will sufficiently decompose the sulfids present therein to enable the precious metals to be readily separated therefrom, then removing the resultant solution and 60 subsequently recovering the precious metals from said material in any convenient manner.

10. The method of treating precious metal bearing materials, containing sulfids, which consists in agitating said material with a 65 suitable gaseous oxidizing agent under pres-

sure in a solution containing a hydroxid of an alkaline earth metal which will sufficiently decompose the sulfids present therein, to enable the precious metals to be readily separated therefrom, then removing the resultant solution, and subsequently recovering the precious metals from said material in any convenient manner. 70

11. The method of treating precious metal bearing materials containing sulfids, which 75 consists in agitating said material with a suitable gaseous oxidizing agent, under pressure with a solution of caustic soda which will sufficiently decompose the sulfids present therein to enable the precious metals to 80 be readily separated therefrom, then removing the resultant solution and subsequently recovering the precious metals from said material in any convenient manner.

12. The method of treating precious metal 85 bearing materials, containing sulfids, which consists in agitating said material with a suitable gaseous oxidizing agent under pressure with a solution containing a carbonate of an alkali metal and caustic soda which 90 will sufficiently decompose the sulfids present therein to enable the precious metals to be readily separated therefrom, then removing the resultant solution, and subsequently recovering the precious metals from said material in any convenient manner. 95

13. The method of treating precious metal bearing materials, containing sulfids, which consists in agitating said material with a suitable gaseous oxidizing agent under pressure 100 in a solution containing a carbonate of an alkali-metal and caustic soda, removing the resultant solution, and subsequently recovering the precious metals from said material in any convenient manner.

14. The method of treating precious metal bearing materials containing sulfids, which consists in agitating said material with atmospheric air under pressure in a basic solution which will sufficiently decompose the 110 sulfids present therein to enable the precious metals to be readily separated therefrom, then removing the resultant solution and subsequently recovering the precious metals from said material in any convenient manner. 115

15. The method of treating precious metal bearing materials containing sulfids, which consists in agitating said material with atmospheric air under pressure in a solution 120 containing alkali-metal which will sufficiently decompose the sulfids present therein to enable the precious metals to be readily separated therefrom, then removing the resultant solution and subsequently recovering 125 the precious metals from said material in any convenient manner.

16. The method of treating precious metal bearing materials containing sulfids, which consists in agitating said material with at- 130

mospheric air under pressure in a solution containing a mixture of a carbonate and a hydroxid of an alkali-metal which will sufficiently decompose the sulfids present therein 5 to enable the precious metals to be readily separated therefrom, then removing the resultant solution and subsequently recovering the precious metals from said material in any convenient manner.

10 17. The method of treating precious metal bearing materials containing sulfids, which consists in agitating said material with atmospheric air under pressure in a solution of caustic soda which will sufficiently decompose the sulfids present therein to enable the precious metals to be readily separated therefrom, then removing the resultant solution and subsequently recovering

the precious metals from said material in any convenient manner.

18. The method of treating precious metal bearing materials, containing sulfids, which consists in agitating said material with atmospheric air under pressure with a solution containing a carbonate of an alkali 25 metal and caustic soda, removing the resultant solution, and subsequently recovering the precious metals from said material in any convenient manner.

In testimony whereof we affix our signatures, in presence of two witnesses.

PAUL W. AVERY.  
EUGENE C. KNOWLES.

Witnesses:

AMOS B. WEST,  
GEO. F. BAGGLEY.